

Feb. 3, 1925.

1,525,027

J. N. EARLY

SAND CASTING

Filed Jan. 10, 1924

Fig. 1



Fig. 2



Fig. 3



INVENTOR  
John N. Early  
By John E. Jackson  
His Attorney.

Patented Feb. 3, 1925.

1,525,027

# UNITED STATES PATENT OFFICE.

JOHN N. EARLY, OF PITTSBURGH, PENNSYLVANIA, ASSIGNOR TO W. J. EARLY SONS FOUNDRY CORPORATION, OF PITTSBURGH, PENNSYLVANIA, A CORPORATION OF DELAWARE.

## SAND CASTING.

Application filed January 10, 1924. Serial No. 685,425.

To all whom it may concern:

Be it known that I, JOHN N. EARLY, a citizen of the United States, and resident of Pittsburgh, in the county of Allegheny, 5 State of Pennsylvania, have invented certain new and useful Improvements in Sand Castings, of which the following is a specification.

This invention relates to an alloy of iron, 10 the main constituents of which are iron, silicon, sulfur, phosphorus, manganese, and carbon, with or without small quantities of nickel and chromium.

This alloy is characterized by having 15 great strength and a very hard chill surface; also by the fact that the chill depth may be readily controlled by the operator, either in a sand or chill mold.

Heretofore, in casting iron alloys the chill 20 depth has been uncontrollable, except by the use of chill pieces or chill molds, and even then has been more or less of an uncertain matter, while the present alloy permits of positive control of the chill depth at all 25 times.

Generically, the invention consists in castings containing the elements and the percentages thereof, following—

|                                        | Per cent.    |
|----------------------------------------|--------------|
| 30 Silicon                             | .75 to 1.50  |
| Sulfur                                 | .05 to .25   |
| Phosphorus                             | .25 to .75   |
| Manganese                              | .20 to .70   |
| 35 Total carbon                        | 2.25 to 3.75 |
| Combined carbon                        | 1.00 to 2.25 |
| Iron, approximately sufficient to make | 100%         |

Such castings show remarkable results in 40 tensile strength and in wearing and abrasive qualities, and in the resistance to the action of heat.

A specific analysis of one of the characteristic castings made under my method 45 and of my new alloy is silicon 1.21%, sulfur .14%, phosphorus .57%, manganese .21%, free carbon 1.76%, and combined carbon 1.54%.

I have discovered that the combined carbon varies more or less in proportion with the sulfur content of the alloy, although some of the other elements may also effect the percentage of combined carbon to a negligible extent.

55 The most notable characteristic of this

new alloy is its ability to chill in either a sand or chill mold, and the ease with which the operator can control the depth of the chill in either a sand mold or chill mold. Rolls for rolling mills, crusher rolls and 60 other castings in which it is desired to have a very hard wear resisting surface may readily be cast in sand molds when formed from my novel alloy and will come out of the mold with a uniform depth of 65 chill of such hardness that they will out-wear ordinary cast rolls from four to five times.

The depth of chill on castings formed from my novel alloy is readily controlled 70 when they are cast in either sand or chill molds by varying the sulfur content and by varying the heat at which the metal is poured into the molds.

Alloys having a high content of combined 75 carbon have been made heretofore, but all of such alloys, such as the well known "adamite," and similar alloys have depended upon the high chromium content to cause the combining of the carbon, while the present alloy has a high combined carbon with 80 or without the use of chromium or nickel.

It will also be noted that due to the peculiar characteristics of "adamite" and similar high chromium alloys, they can not 85 be produced commercially in a cupola, while the present alloy may readily be produced in a cupola, electric furnace, or other smelting furnace. In fact, for several months past the alloy of this invention has been 90 commercially produced in a cupola.

When it is desired to increase the tensile strength and toughness of the castings, I 95 may add a relatively small amount of chromium and nickel, as for instance, chromium .15% to .25% and nickel .05% to .25%. It will be noted, however, that when either chromium or nickel alone, or both together are added to my alloy, the percentage of combined carbon remains substantially the same.

In producing my novel alloy, the following method is carried out—

I first charge a cupola or other smelting furnace with suitable scrap, pigs, or ores, 105 of the proper analysis to enable me to secure the proper proportion of silicon, sulfur, phosphorus, manganese, and carbon, and if chromium and nickel are to be included in the alloy, suitable pigs contain- 110

ing these ingredients are also added. After the mix is made up it is heated to from 2500 degrees to 2700 degrees Fahrenheit to melt the metals. That is, the mix is raised 5 to a heat materially above the melting temperature so as to obtain a good pouring temperature. After the mix has been melted it is tapped and then poured in the molds at a temperature of from 2300 degrees to 10 2500 degrees Fahrenheit.

The depth of chill on the finished casting is controlled primarily by the pouring temperature. That is, the hotter the pouring temperature the deeper will be the chill; 15 also the depth of chill can be controlled somewhat by the sulfur content of the mix, that is, the greater the sulfur content the greater the chill. However, the sulfur content is known and when it is 20 slightly higher or lower than necessary to produce the correct depth of chill, the pouring temperature may be increased or lowered accordingly to give the correct depth of chill.

25 For instance, if the sulfur content were such that it would tend to cause too great a depth of chill, then the pouring temperature would be lowered to lessen the chilling effect of the casting heat, while if the sulfur content was slightly lower than necessary to give the desired depth of chill, the pouring heat would be increased.

This alloy is peculiar to itself in that it 30 will form a uniform depth of chill over the entire surface of a casting in a sand mold, and the depth of such chill can be varied or controlled by the pouring temperature, so that an operator may readily produce castings such as crusher rolls, dies, 35 rolling mill rolls, rolling mill guides, etc., with definite depths of chill over their entire surface.

40 Experience has shown that crusher rolls, rolling mill guides, dies and other castings formed from my alloy will outlast as many as four or five similar articles made from ordinary cast iron alloys or steels. The chilled surfaces of articles made from my alloy are very hard and will outwear any 45 commercial steel or iron alloy known at this time. In fact, in most cases it is so hard that it will withstand any of the commercial forms of tool steel and cannot be turned on a lathe, but must be ground to 50 finish.

55 Referring to the accompanying drawings, Figure 1 is a transverse elevation through a rolling mill roll.

60 Figure 2 is a transverse section through a rolling mill guide.

65 Figure 3 is a transverse section through a small round cast bar.

Referring particularly to the drawings, the numeral 2 in each of the above figures designates the hard uniform chilled outer surface of the castings and the numeral 3 designates the soft or unchilled center. All 65 of the above articles can and are produced in the well known sand mold and their chill depth has been produced without the 70 use of any form of chill pieces or mold.

The uniformity of the chill is due to the novel composition of my new alloy and the depth of the chill is controlled by the pouring temperature so that the operator after 75 little experience may readily make chill depths of from one-eighth or less to one and one-half or more inches from the same alloy mix by simply varying the pouring temperature.

80 Applicant believes he is the first to produce an iron alloy capable of being cast in sand and to produce a uniform depth of chill without the use of chill molds or chill pieces, and therefore, does not wish to be limited to the exact articles shown and described, but intends his claims to be construed broadly so as to include any article 85 cast in sand from his or the equivalent of his alloy, which is provided with a uniform depth of chill.

90 I claim—

95 1. As an article of manufacture a sand casting having a uniform chill depth over its entire surface and an unchilled center.

100 2. As an article of manufacture a sand casting having a uniform chill depth over its entire surface and an unchilled center, said chilled surface being characterized by being of such hardness that it can not be 100 cut by the commercial forms of tool steel.

105 3. As an article of manufacture a sand cast roll for rolling mills and the like having a uniform chill depth over its entire surface and an unchilled center.

110 4. As an article of manufacture a sand casting of iron alloy comprising essentially silicon .75% to 1.50%; sulfur .05% to .25%; phosphorus .25% to .75%; manganese .20% to .70%; combined carbon of from 1.00% to 2.00%; some free carbon; and iron approximately sufficient to complete the 100%, said casting being characterized by having a uniform chill depth over its entire surface and an unchilled center, the depth of 115 said chill being under the control of the operator due to the peculiar characteristic of the alloy which permits the control of the chill by varying either the sulfur content or the pouring temperature, or both.

120 In testimony whereof, I have hereunto signed my name.

JOHN N. EARLY.